

1

2,742,340

## VAT DYEING PROCESS

Donald E. Marnon, Glen Rock, N. J., assignor to General Aniline & Film Corporation, New York, N. Y., a corporation of Delaware

No Drawing. Application September 6, 1951,  
Serial No. 245,423

12 Claims. (Cl. 8—34)

This invention relates to an improved method of dyeing with vat dyes and more particularly to a high temperature vat dyeing process.

Since the advent of high speed, high temperature, continuous dyeing, a new requirement has been imposed on vat dyes, namely, one of stability in their leuco form to temperatures approaching the boil. Many vat dye colors, otherwise highly desirable because of their particular shade, fastness, and other properties have been found to be unstable at the temperatures employed in many of the newly developed vat dyeing processes. This sensitivity to high temperatures results in dyeings which are uneven, specky and weak and, in general, of an uneven and inferior shade. This may be due to over-reduction or incomplete reduction of the vat dyestuff, instability and decomposition at the high temperatures, etc.

According to one aspect of the present invention, it has been found that the defects occurring when dyeing with thermally unstable vat dyes in leuco form, particularly at temperatures ranging from about 150° to 220° F., may be corrected by maintaining the reduction potential in the leuco dye bath at a predetermined optimum value by the gradual controlled addition to the dye bath of appropriate reducing substances, stabilizing substances and alkali. It will of course be understood that this process may be employed in applying any leuco vat dyes at any suitable temperatures. The process is followed by the usual finishing or oxidizing treatments. The term "dye bath" in this disclosure and the appended claims is employed to include the usual bath containing a solution of the vat dyestuff in reduced leuco and in which the fibrous material is dyed, and also those cases in which fibrous material is first padded or impregnated with the dyestuff and then treated with a reducing material in another operation. In the latter case, the bath at or in the fiber contains both the reducing substance and the dyestuff, and is thus essentially a "dye bath."

As suitable reducing substances may be mentioned sodium hydrosulfite and other substances well known in the vat dyeing art for reducing vat dyes to their leuco form. As suitable stabilizing substances may be mentioned sugars, dextrans, inorganic nitrites and other substances whose reduction potentials do not exceed that of the reducing substance employed. It will be understood that other agents may be added to the aforementioned substances for their known functions, such as salt and the like.

It has been found that at reduction potentials below about 750 mv. (when measured by means of a saturated calomel-platinum electrode system) dyeings may be obtained which are uneven, specky and weak due to the incomplete reduction of the vat dyestuff and in such cases an increase in the amount of reducing substances added is called for. At reduction potentials greater than about 1,100 mv. the shade may become inferior, presumably due to over-reduction of the vat dyestuff which would tend toward oxanthrone formation, particularly in the case of Indanthrene Blue BC (C1113) which dye-

2

stuff, while yielding a most desirable shade, has been found to be particularly sensitive to high temperatures. In such cases, of course, the addition of stabilizing substances is called for. The preferred reduction potential range is in most cases about 930 to 1050 mv.

Fibrous materials to which the process is applicable are all those materials which are susceptible to coloration by vat dyeing processes. Such materials may be in any suitable form, as for example, fabrics, yarns, ropes, warps, fibers, filaments and the like.

The process is applicable to various types of vat dyeing methods, as for example, continuous dyeing, jig dyeing (piece work), Beck open vat dyeing, package dyeing, and the like.

The instant invention is applicable to vat dyeing processes in general, employing any suitable temperatures and pressures, but it is most effective in the high temperature application of thermally unstable vat dyestuffs such as the dianthraquinone dihydroazines. Thus, the process is also advantageously employed in applying dyestuffs such as Indanthrene Blue BFP (CI 1113), Algol Orange RF (CI 1217), Indanthrene Brilliant Violet 2R (CI 1104), Indanthrene Blue RS (CI 1106), Indanthrene Blue GC (CI 1112), Indanthrene Olive R (CI 1150), 2,28-diethyl-2, 2'-bianthra [1,9] pyrazole-6,6'(2H,2'H)-dione, 4,10-dibromodibenzo [c, d, j, k] pyrene-6,12-dione, tetrabromo - 8,16 - pyranthrenedione, trichloro - N,N'-diphenyl-3,4,9, 10-perylene-tetracarboxylic dimide, 3-(1-anthraquinononylamo) antha [9, 2, 1-a m n] naphth [2, 3-h] acridine-5, 10, 15 (16H)-trione and the products disclosed in U. S. Patents 1,706,902; 1,758,365; 1,790,780; 1,790,843; 1,803,757; 1,832,209; 1,845,469; 1,851,082; 1,877,315; 1,877,945; 1,885,172; 1,904,145; 1,931,821; 1,943,710; 1,945,484; 1,949,209; 2,086,843; 2,118,192; 2,123,251; 2,228,445; 2,238,209 and mixtures thereof.

The control of the reduction potential of the dye bath can be maintained by following the course of the reduction with a calomel-platinum electrode system in turn connected to a recording potentiometer. By means of this system, one is able to anticipate the need for either reducing agent or protective agent depending on the measured reduction potential. The control of the feed of the alkali, reducing agent and stabilizing agent may be manual or automatic and, of course, automatic control is preferable where possible. By way of example, the recording potentiometer may be connected through automatic control means well known per se to separate feed systems for the alkali-sodium hydrosulfite or other reducing agent and for the dextrin, sodium nitrite or other stabilizing or protecting agent in such a manner that when the measured reduction potential exceeds the optimum predetermined value for the particular type of dyeing being carried out, the stabilizing agent feed is activated or increased and when the measured reduction potential falls below the optimum value, the reducing agent feed is activated or increased. The reducing agent, such as sodium hydrosulfite, is ordinarily added together with a predetermined amount of caustic, potash, or the like. In some instances, however, the reducing agent alone may be added when needed to keep the reduction potential of the bath at the optimum predetermined value, and alkali added only when it is found that addition of the reducing agent alone does not produce the desired increase in reduction potential. The reducing material may comprise a mixture of reducing agents, and similarly, the stabilizing or protective material may comprise a mixture of stabilizing agents. In some cases it is preferable to add the reducing and stabilizing agents together in one mixture, and in such cases, the mixture is only added to the dye bath or reducing bath when the measured reduction potential falls below the optimum predetermined value for producing the desired results.

It will of course be understood that although the above described saturated calomel-platinum electrode system is preferred for measurement of the reduction potential in accordance with the invention, other suitable systems may be used. While the millivolt values of the reduction potential measured by other systems may, because of use of different reference electrodes or other causes, differ from the values recommended hereinbefore, it should be apparent that the actual value of the reduction potential to be employed in any particular instance for obtaining the best results will be the same regardless of the measuring system employed. Accordingly, the operative reduction potential range for use in the present invention may be expressed as a value equivalent to from about 750 to 1100 mv. when measured by means of a saturated calomel-platinum electrode system.

The use of soluble inorganic nitrites, particularly sodium nitrite, as stabilizing substances in vat dye baths to prevent over-reduction has been recently proposed. It has been found however that use of these nitrites is attended with various difficulties, chief among which is the fact that their full protective or stabilizing action is only developed in the bath after reduction has proceeded for some time. This lag in the stabilizing activity of the nitrites results in over-reduction of the initial portions of the dyed fibrous material. Nor can this difficulty be readily corrected by the practice of initially charging increased amounts of nitrite (up to 500% or more of the amount of nitrite otherwise required), since although this remedies the aforementioned initial over-reduction, the increased stabilizing or protective activity later developed so retards proper reduction of the dyestuff that subsequent portions of the dyed fibrous material are found to be incompletely reduced. These difficulties are especially pronounced in the case of many presently employed rapid continuous dyeing processes, in which uniform level dyeings from the beginning to the end of the runs may not thereby be obtained.

Applicant has made the discovery that the aforementioned difficulty in obtaining adequate protective or stabilizing action against initial over-reduction may be remedied by initially charging hydroxylamine into the dye bath in addition to the amount of nitrite found to be sufficient for the subsequent stabilization or protection of the reducing process. In this manner initial and subsequent protection is obtained, with consequent advantageous results with respect to the dyeings produced.

The hydroxylamine is preferably added in the form of its salts, as for example hydroxylammonium sulfate, hydroxylammonium acid sulfate, hydroxylammonium hydrochloride and the like, in molar ratios of nitrite to hydroxylamine of from about 1:2 to 4:1.

The above described process has been found to remove the difficulties previously met with in the employment of high temperature vat dyeing processes but further, it has been found that by the process of the invention, remarkable savings in the amounts of materials used is effected. This is made possible by the fact that the exact amounts of materials necessary for replenishing the bath to maintain its reducing action may be thus instantaneously determined and added as needed. The excess material usually added as a safety factor to allow for errors caused by the heretofore relatively crude estimations of the requirements of the dye bath based on resultant shades and past experience is thereby saved. The dyeings obtained are uniform and highly acceptable from both a scientific and commercial aspect.

The following examples are merely illustrative of the invention and are not to be regarded as limitative:

#### Example 1

A stirred solution of 10 oz. sodium hydroxide in 2½ gallons of water was heated to 180° F. and 2½ oz. Indanthrene Blue BFP (dichloro dianthraquinone dihydro-

azine) were added. After a few minutes the dyestuff was dispersed. Two electrodes for measurement of the oxidation-reduction potentials were inserted in the bath (the electrodes were a measuring [platinum] electrode and a saturated calomel [mercury-mercurous chloride-saturated KCl] reference electrode).

At zero minutes there were added 213 g. of dextrin and 142 g. of sodium hydrosulfite, and the reduction potential as measured by a Beckman pH meter (whose range had been extended by the addition of a "bucking" potential) and recorded on a Brown recorder was found to be 972 mv. The Beckman pH meter is a well known high input impedance indicator.

After five minutes, the potential had gradually dropped to 964 mv. The potential was maintained at about 180° F. for 90 minutes between 950 and 960 millivolts by the addition of dry hydrosulfite (total 240 g. in almost a continuous manner) and dextrin (total 160 g. in 10 g. portions). Addition of hydrosulfite increased the reduction potential while addition of dextrin impeded increase of the reduction potential. In this experiment dextrin was added when the potential increased to 955 or 960 mv.

Cotton swatches (8 dyeings) were dyed at about ten minute intervals. The swatches were found to be dyed uniformly when the potential was held in the range of 950-960 mv.

#### Example 2

A mill trial involving 2,000 yards of cloth was carried out under the following conditions:

White broadcloth was padded through a suspension of Ind. Blue BFP (1 lb./gal.), squeezed and then developed continuously in a Williams Unit (see U. S. Patent 2,364,838) containing the following initial charge:

3½ oz./gal. sodium hydroxide  
3½ oz./gal. sodium hydrosulfite  
0.2 oz./gal. hydroxylammonium sulfate  
0.2 oz./gal. sodium nitrite  
0.26 oz./gal. Ind. Blue BFP

A temperature of 200-208° F. was maintained throughout the run. The potential measured as in Example 1 was 1025 mv. The potential was maintained throughout the run by a variable feed (2-5 gal./min.) of a feed liquor composed as follows:

3½ oz./gal. sodium hydroxide  
3½ oz./gal. sodium hydrosulfite  
0.2 oz./gal. sodium nitrite

The cloth was then finished in the usual manner. Shading of the material was excellent.

#### Example 3

The procedure of Example 2 was repeated on a 7,000 yd. run of a lighter shade as follows:

Conc. of pad bath:

0.87 oz./gal. Ind. Blue BFP  
0.125 oz./gal. dimethoxyviolanthrone

Composition of developing bath:

1.53 oz./gal. sodium hydroxide  
1.4 oz./gal. sodium hydrosulfite  
0.1 oz./gal. hydroxylammonium sulfate  
0.1 oz./gal. sodium nitrite  
0.014 oz./gal. Ind. Blue BFP  
0.002 oz./gal. dimethoxyviolanthrone

Composition of feed (2 gal./min.):

2.5 oz./gal. sodium hydroxide  
2.5 oz./gal. sodium hydrosulfite  
0.1 oz./gal. sodium nitrite

In this case a potential of 940-955 mv. measured as in Example 1 was maintained at 200 to 205° F. Again this cloth was finished in the usual manner. Shading

was excellent and the amounts of chemicals required were  $\frac{1}{3}$  of the usual amount.

In the instant example and in the previous example, dyestuff was added to the initial charge to prevent "tailing" or stripping of padded dyestuff from initial portions of the goods and deposition on subsequent portions, which would result in a non-uniform dyeing.

*Example 4*

A mill trial involving 750 yards of Fortisan (stretched, saponified cellulose acetate) was carried out under the following conditions:

26 lbs. of a vat dyestuff of the formula:



9 lbs. 12 oz. of a vat dyestuff of the formula:



1 lb. 10 oz. of Ind. Golden Orange GA Double Paste (CI 1096) were vatted with 14 lbs. sodium hydroxide and 14 lbs. sodium hydrosulfite in 110 gal. H<sub>2</sub>O for 10 minutes at 120° F.

The resulting vat was used to dye 750 yards of Fortisan (prepared for dyeing by a brief pretreatment in 6% caustic solution at 60–70 F.) on a jig for 8 ends at 15 minutes per end. The first two ends were run at 120° F. and the last six ends at 130° F. A reduction

potential of 990–1025 mv. measured as in Example 1 was maintained throughout the runs by adding

4 lbs. sodium hydroxide and  
7 lbs. sodium hydrosulfite

in increments as needed. In this example, the hydrosulfite was added separately when needed to maintain the reduction potential up to the required value. When further addition of hydrosulfite alone had no effect on the reduction potential, caustic was added to replenish the bath. This method of feed was found to be more convenient and desirable than continued addition of caustic and hydrosulfite together in predetermined proportions.

The dyeing obtained was of excellent quality, shade, fastness, levelness and uniformity.

Various modifications and variations of this invention will be obvious to a person skilled in the art and such variations and modifications are to be regarded as within the purview of this application and the spirit and scope of the appended claims.

I claim:

1. In a process of vat dyeing fibrous materials in a vat containing dyestuff, a reducing substance therefor, alkali, and an inorganic nitrite, the improvement comprising initially adding hydroxylamine to the vat in a molar ratio of nitrite to hydroxylamine of from about 1:2 to 4:1.

2. A continuous process for vat dyeing fibrous materials comprising the steps of impregnating the fibrous material with vat dyestuff, passing the fibrous material continuously through a reducing bath containing caustic, sodium hydrosulfite, sodium nitrite and hydroxylamine, and continuously replenishing the reducing bath with a supply of caustic, sodium hydrosulfite and sodium nitrite.

3. In a process of vat dyeing fibrous materials, the improvement comprising maintaining the reduction potential, during dyeing, in the dyebath, which has been initially charged with vat dyestuff, reducing substance, sodium nitrite, and hydroxylamine, at a value equivalent to from about 750 to 1100 mv. when measured by means of a saturated calomel-platinum electrode system connected to a high input impedance indicator by the gradual controlled addition to the dyebath of a reducing substance and sodium nitrite.

4. The process of claim 3 wherein the sodium nitrite and hydroxylamine in the initial charge are in a molar ratio of from about 1:2 to 4:1.

5. In a process of vat dyeing fibrous materials, the improvement comprising maintaining the reduction potential, during dyeing, in the dyebath, which has been initially charged with vat dyestuff, reducing substance, sodium nitrite, and hydroxylamine, at a value equivalent to from about 750 to 1100 mv. when measured by means of a saturated calomel-platinum electrode system connected to a high point input impedance indicator by continuously measuring the reduction potential in the dyebath, and by adding a reducing substance and sodium nitrite when the measured potential falls below the desired value.

6. The process of claim 5 wherein the sodium nitrite and hydroxylamine in the initial charge are in a molar ratio of from about 1:2 to 4:1.

7. In a process of vat dyeing fibrous materials, the improvement comprising maintaining the reduction potential, during dyeing, in the dyebath, which has been initially charged with vat dyestuff, reducing substance, sodium nitrite, and hydroxylamine, at a value of from about 750 to 1100 mv. by continuously measuring the reduction potential in the dyebath by means of a saturated calomel-platinum electrode system connected to a high input impedance indicator and by adding a reducing substance and sodium nitrite when the measured potential falls below the desired value.

8. The process of claim 7 wherein the sodium nitrite

and hydroxylamine in the initial charge are in a molar ratio of from about 1:2 to 4:1.

9. In a process of vat dyeing fibrous materials by impregnating with dichloro dianthraquinone dihydroazine and reducing at a temperature of from 200 to 208° F. the improvement comprising maintaining the reduction potential, during dyeing, in the reducing bath which has been initially charged with said dyestuff, caustic, sodium hydro sulfite, sodium nitrite and hydroxylamine at about 1025 mv. by continuously measuring the reduction potential therein by means of a saturated calomel-platinum-electrode system connected to a high input impedance indicator and adding caustic, sodium hydro sulfite and sodium nitrite when the measured potential falls below about 1025 mv.

10. The process of claim 9 wherein the sodium nitrite and hydroxylamine in the initial charge are in a molar ratio of from about 1:2 to 4:1.

11. In a process of vat dyeing fibrous materials by impregnating with a mixture of dichloro dianthraquinone dihydroazine and dimethoxyviolanthrone and reducing at a temperature from about 200 to 205° F., the improvement comprising maintaining the reduction potential dur-

ing dyeing in the reducing bath which has been initially charged with said vat dyestuffs, caustic, sodium hydro sulfite, sodium nitrite and hydroxylamine at from about 940 to 955 mv. by continuously measuring the reduction potential therein by means of a saturated calomel-platinum-electrode system connected to a high input impedance indicator and adding caustic, sodium hydro sulfite and sodium nitrite when the measured potential tends to fall below 940 mv.

10 12. The process of claim 11 wherein the sodium nitrite and hydroxylamine in the initial charge are in a molar ratio of from about 1:2 to 4:1.

References Cited in the file of this patent

UNITED STATES PATENTS

|           |       |       |               |
|-----------|-------|-------|---------------|
| 2,548,543 | Mecco | ----- | Apr. 10, 1951 |
| 2,548,545 | Mecco | ----- | Apr. 10, 1951 |
| 2,576,846 | Mecco | ----- | Nov. 27, 1951 |

OTHER REFERENCES

American Dyestuff Reporter for December 12, 1949, pgs. P919 to P922, inclusive.